

[54] NICEL-IRON MAGNETIC ALLOYS  
COMPRISING CHROMIUM AND  
MOLYBDENUM

[75] Inventor: Nobukazu Kuroda, Kanagawa-ken,  
Japan

[73] Assignee: Sony Corporation, Tokyo, Japan

[22] Filed: Jan. 19, 1973

[21] Appl. No.: 325,144

[30] Foreign Application Priority Data

Jan. 27, 1972 Japan..... 47-010146

[52] U.S. Cl..... 148/31.55, 75/170, 75/171,  
148/108

[51] Int. Cl..... C04b 35/00

[58] Field of Search ..... 148/31.55, 108; 179/100.2;  
340/174 TF, 174 NA; 75/170, 171

[56] References Cited

UNITED STATES PATENTS

|           |         |                    |           |
|-----------|---------|--------------------|-----------|
| 1,910,309 | 5/1933  | Smith et al.....   | 75/170    |
| 2,891,883 | 6/1959  | Howe.....          | 75/170    |
| 3,024,142 | 3/1962  | Parkin.....        | 75/170    |
| 3,575,734 | 4/1971  | Muzyka et al. .... | 75/170    |
| 3,582,408 | 6/1971  | Onyshkevych.....   | 148/31.55 |
| 3,698,055 | 10/1972 | Holtz et al. ....  | 75/170    |

Primary Examiner—Walter R. Satterfield  
Attorney, Agent, or Firm—Hill, Gross, Simpson, Van  
Santen, Steadman, Chiara & Simpson

[57] ABSTRACT

Magnetic alloys comprised of iron, nickel, chromium  
and molybdenum in which a weight ratio of nickel to  
iron is selected in a range of about 0.54 to 1.5.

4 Claims, 15 Drawing Figures

PATENTED OCT 29 1974

3,844,849

SHEET 1 OF 8

FIG - 1



FIG - 2



FIG. 2 - 3







PATENTED OCT 29 1874

3,844,849

SHEET 6 OF 8

Fig. 9.



PATENTED OCT 29 1974

3,844,849

SHEET 7 OF 8



SHEET 8 OF 8

 $10\mu$   
0.5mmFig - 12A

—case—|—core—|—case—|—core—|

Fig - 12B

—case—|—core—|—case—|—core—|

Fig - 12C

—case—|—core—|—case—|—core—|

Fig - 12D

—case—|—core—|—case—|—core—|



# NICKEL-IRON MAGNETIC ALLOYS COMPRISING CHROMIUM AND MOLYBDENUM

## BACKGROUND OF THE INVENTION

### 1. Field of the Invention

The present invention relates generally to magnetic alloys and more particularly to magnetic alloys which are useful as magnetic shield material for magnetic heads.

### 2. Description of the Prior Art

Generally, magnetic shield materials for a magnetic head have been formed of an iron-nickel binary alloy consisting of 79 weight percent nickel and 21 weight percent iron, that is, a so-called 79-Permalloy. The 79-Permalloy has magnetic characteristics whereby its initial permeability is more than 3,000 and its magnetic flux density is more than 3,000 Gausses. Such magnetic characteristics are most preferable for a magnetic shield material that is to be used in combination with a magnetic head. Such a 79-Permalloy, however, has the drawback that its manufacturing cost is rather high due to the fact that it is difficult to work during manufacturing processes and that it contains a large amount of nickel which is uneconomical.

45-Permalloy (containing 45 weight percent nickel and 55 weight percent iron) has been also proposed, which is relatively easily processed during manufacturing due to the fact that it contains less nickel but has enough magnetic characteristics to function as a magnetic shield material for a magnetic head. However, rust is apt to be formed on such 45-Permalloy. In other words, rust is gathered on a shield case or plate made of 45-Permalloy during a rinsing step in a typical manufacturing process or after manufacturing, so that 45-Permalloy is not practically useful.

Further, both of the 79-Permalloy and 45-Permalloy are about 120-130 in hardness (Vickers scale) and show poor wear resistance. For this reason, a magnetic shield and/or head composed of such Permalloys has a short life time and is undesirable for use in magnetic recording and/or reproducing on and/or with a magnetic tape using chromium dioxide powders.

## SUMMARY OF THE INVENTION

The present invention provides a magnetic shield material wherein a part of the iron or the nickel content in an iron-nickel alloy is substituted by chromium and molybdenum to provide an iron-nickel-chromium-molybdenum quadruple or quaternary alloy, by which the drawbacks encountered in the prior art are avoided.

Accordingly, it is an object of the present invention to provide magnetic alloys which are easily rolled or worked and manufactured at low cost.

It is a further object of the present invention to provide a magnetic alloy which is high in wear resistance and suitable as a magnetic shield material for a magnetic head.

It is a yet further object of the present invention to provide an anti-corrosive or anti-rust magnetic alloy which is manufactured at low cost.

The other objects, features and advantages of the present invention will be apparent from the following description taken in conjunction with the accompanying drawings.

## BRIEF DESCRIPTION OF THE DRAWINGS

FIG. 1 is a graph showing a characteristic or relationship between the amount of chromium (Cr) added to an iron-nickel (FeNi) alloy and the initial permeability of thus obtained alloy;

FIG. 2 is a graph showing a characteristic or relationship between the amount of molybdenum (Mo) added to an iron-nickel alloy and the initial permeability of thus obtained alloy;

FIG. 3 is a graph showing relationship between amounts of Cr, Mo and Ni added to ternary alloys of (FeNi)Cr, (FeNi)Mo and a binary alloy (FeNi)Ni, respectively, and the rust forming rates of thus manufactured alloys;

FIG. 4 is a graph showing relationship between the ratio of Ni/Fe in a ternary alloy (FeNi)Cr and the amount of Cr therein at a critical point where the rust disappears during rust forming test in salt water;

FIG. 5 is a graph showing a characteristic curve which illustrates the state of magnetic flux modification produced by changing the amount of Ni in an FeNi alloy;

FIG. 6 is a graph showing magnetic characteristic curves, such as the initial permeability  $\mu_0$ , maximum magnetic flux density B, and coercive force Hc, relative to the amount of Cr in a ternary alloy  $(Fe_{60}Ni_{40})_{1-x}Cr_x$ ;

FIG. 7 is a graph showing magnetic characteristic curves, such as the initial permeability  $\mu_0$ , maximum magnetic flux density B, and coercive force Hc relative to the amount of Mo in a ternary alloy  $(Fe_{60}Ni_{40})_{1-x}Mo_x$ ;

FIG. 8 is a composition diagram showing rust forming rate of quadruple or quaternary alloy (FeNi)CrMo relative to the amounts of Cr and Mo therein;

FIG. 9 is a composition diagram showing the magnetic permeability  $\mu_0$ , coercive force Hc, and magnetic flux density B of a quadruple alloy (FeNi)CrMo relative to the amounts of Cr and Mo therein;

FIG. 10 is a graph showing magnetic characteristics, such as the magnetic permeability  $\mu_0$ , coercive force Hc, and magnetic flux density B of a quadruple alloy  $(Fe_{60}Ni_{40})_{92-x}Cr_xMo_x$  relative to the amount of Mo therein;

FIG. 11 is a perspective view of a magnetic head using the magnetic alloys according to the present invention; and

FIGS. 12A to 12D inclusively, are cross-sectional views, respectively, illustrating surface conditions of the magnetic head depicted in FIG. 11 after a wear test thereof wherein the shield case and magnetic core of the magnetic head are changed in composition.

## DESCRIPTION OF THE PREFERRED EMBODIMENTS

It has been discovered that when chromium (Cr), which improves anti-corrosive characteristics of magnetic material, and molybdenum (Mo), which enhances permeability of magnetic material, are added to a composition consisting mainly of iron (Fe) and nickel (Ni) in small but definite amounts, a magnetic alloy high in permeability can be obtained even if the amount of nickel is reduced therein.

A magnetic alloy according to the present invention comprises a magnetically heat-treated alloy composed of about 6 to 12 weight percent of chromium (Cr),

about 0.5 to 8 weight percent of molybdenum (Mo), and the balance of iron (Fe) and nickel (Ni) in which the ratio of nickel (Ni) to iron (Fe) is selected from about 0.54 to about 1.5. The magnetic alloy of the invention has the necessary magnetic flux density and initial permeability required for a magnetic shield material for a magnetic head.

The magnetic alloys of the invention will be illustrated by various exemplary embodiments set forth hereinafter and their characteristics will be compared to certain other compositions so that those skilled in the art may undertake various alterations and modifications to arrive at a particularly desired magnetic alloy composition.

FIGS. 1 to 10 inclusive, are, respectively, graphs or diagrams which show the results of experiments carried out for determining the preferred compositions of magnetic alloys in accordance with the principles of the invention.

FIGS. 1 and 2, respectively, show the relationship between the amounts of chromium (Cr) and molybdenum (Mo) added to an iron-nickel (FeNi) alloy and initial permeabilities of the alloys thus obtained.

FIG. 1 is a graph showing the relationship between the amount of Cr (by weight percent added to an FeNi alloy and the initial permeability  $\mu_0$  of a ternary alloy FeNiCr thus obtained. In the graph of FIG. 1, the abscissa represents the amount of Cr in weight percent and the ordinate represents the initial permeability,  $\mu_0$ . In this example, the amount of Fe was selected to be substantially equal to that of Ni in weight percent. From the characteristic curve, namely the relationship shown in FIG. 1, it will be observed that as the amount of Cr added to the FeNi alloy increases, the initial permeability  $\mu_0$  of FeNiCr alloy decreases.

FIG. 2 is a graph showing the relationship between the amount of Mo added to an FeNi alloy in which the amount of Fe was selected substantially equal to that of Ni in weight percent and the initial permeability,  $\mu_0$  of the resultant FeNiMo alloy. It will be observed from the characteristic curve, namely the relationship depicted in FIG. 2, that even if Mo is added to the FeNi alloy in relatively small amounts, the FeNiMo alloy has an initial permeability,  $\mu_0$  higher than that of the FeNiCr alloy by about a factor of 10.

FIG. 3 is a graph for showing the relationship between the rust forming rates in the alloys represented by (FeNi)Cr at curve I, (FeNi)Mo at curve II and (FeNi)Ni at curve III with various amounts of Cr, Mo and Ni when the alloys were heated at 600° C. in air. In this graph, the abscissa represents the amounts of Cr, Mo, and Ni, respectively, while the ordinate shows the rust forming rates. In this example, the amounts of Fe and Ni were substantially equal in each case. In the graph of FIG. 3, the dotted-line curve IV represents the similar relationship of the binary alloy Fe<sub>50</sub>Ni<sub>50</sub>. Marked solid points on these curves show the composition where rust was formed on the alloys, which were immersed in salt water of 8 percent and 1.5 percent; marked points having an asterisk show the compositions where rust was formed on the alloys, which were immersed in salt water of 8 percent in 200 hours; and marked circles show the compositions where no rust was formed on the alloys, which were immersed in salt water mentioned above. The rust forming rate on the ordinate is designated K where  $m = \sqrt{Kt}$  and  $m$  represents the weight of rust formed and  $t$  represents a time

period during which the alloys were heated at 600° C. in air, while the abscissa represents the adding rate of the alloy materials, namely, Cr, Mo and Ni by weight percent. As is apparent from FIG. 3, an alloy having high anticorrosive characteristics is attained when various amounts of Cr are added thereto.

FIG. 4 is a graph showing a characteristic curve  $a$  between a ratio of Ni to Fe in weight percent, namely, the ratio Ni<sub>y</sub>/Fe<sub>1-y</sub> and the critical amount  $x$  (in weight percent) of Cr, where no rust is formed on the alloy of such a composition as represented by the formula (Fe<sub>1-y</sub>Ni<sub>y</sub>)<sub>1-x</sub>Cr<sub>x</sub> which is immersed in salt water. In this case, the critical amount where no rust is formed is taken as the rust forming rate K of the 79-Permalloy, which has been employed widely as material for a magnetic head and is known not to present a problem of forming rust in practical use. This standardized rust forming rate K is equal to 0.01. It is, of course, desirable that a select material of the invention have a rust forming rate K smaller than 0.01. In FIG. 4, the ordinate represents the amount of Cr in weight percent and the abscissa ratio of Ni<sub>y</sub>/Fe<sub>1-y</sub> in weight percent. The scale 0.54 on the abscissa shows the composition of Fe<sub>65</sub>Ni<sub>35</sub>, the scale 1.0 the composition of Fe<sub>50</sub>Ni<sub>50</sub> and the scale 1.5 the composition of Fe<sub>40</sub>Ni<sub>60</sub>, respectively.

In the graph of FIG. 4, the area (1) under the characteristic curve  $a$  shows an area where rust tends to form on the alloys represented by the compositions in this area. Rust hardly forms on alloys represented by the compositions in the area (2) above the characteristic curve  $a$ .

As will be noted from FIG. 4, in compositions where the value of the ratio Ni<sub>y</sub>/Fe<sub>1-y</sub> is greater than 1.5, that is to say, the amount of Ni to that of Fe is greater than 60 weight percent, no rust is formed on the alloy, unless an amount of Cr is added thereto. Accordingly, with the present invention the rust characteristic is improved by reducing the amount of Ni, which is uneconomical and by adding an amount of Cr. Further, since Mo contributes less to the improvement of the rust repelling characteristic of the alloy, the ratio of Ni/Fe in the binary alloy FeNi is selected smaller than 1.5, for example, as in Fe<sub>40</sub>Ni<sub>60</sub>.

On the other hand, the alloy of FeNi is mainly divided into two phases, one of which is in the phase of iron Fe containing Ni from 0 to 30 weight percent, as seen from FIG. 4 above, and the other phase is in the phase of nickel Ni containing Ni from 40 to 100 weight percent. In the former phase (within the range containing Ni from 0 to 30 weight percent), the alloy has the crystal structure of body center cubic lattice at low temperature but at high temperature it is transformed into a crystal structure of face center cubic lattice, while in the latter phase (within the range containing Ni from 40 to 100 weight percent), the alloy becomes a solid solution of face center cubic lattice irrespective of temperature. On the boundary (Ni being 30-40 weight percent) between such two phases, the saturation magnetization of the alloy is lowered slightly and at the same time its Curie point is greatly lowered, so that its magnetic flux density B is also greatly lowered at room temperature. Accordingly, the alloy becomes substantially non-magnetic, and this characteristic is illustrated in FIG. 5. Even when attempts to increase the magnetic flux density B from the point mentioned above are tried, by adding Mo thereto, at least the alloy FeNi

must contain more than 35 weight percent of Ni and hence the ratio of Ni/Fe in weight percent must be at least 0.54, that is to say,  $Fe_{65}Ni_{35}$  or more as shown at FIG. 4.

FIG. 6 is a graph showing the relationship between the initial permeability  $\mu_0$ , magnetic flux density B, and coercive force Hc, of a ternary alloy  $(FeNi)_{1-x}Cr_x$  (along the ordinate) and where the amount x of Cr contained therein is changed and the alloy FeNi is selected to be  $Fe_{60}Ni_{40}$ , which is the ratio of Ni/Fe slightly greater than that of the FeNi alloy which has a greatly decreased magnetic flux density B, as described just above in conjunction with FIG. 5. In the graph of FIG. 6, reference numeral I represents the curve of the initial permeability  $\mu_0$ ; numeral II represents the curve of the magnetic flux density B, and numeral III represents the curve of the coercive force Hc, respectively.

FIG. 7 is a graph illustrating the relationship between the initial permeability  $\mu_0$ , the magnetic flux density B, and the coercive force Hc of a ternary alloy  $(FeNi)_{1-x}Mo_x$  and where the amount x of Mo contained therein is changed and the alloy FeNi is also selected to be  $Fe_{60}Ni_{40}$ , as in the compositions of FIG. 6. In the graph of FIG. 7, curve I shows the initial permeability  $\mu_0$ , curve II the magnetic flux density B and curve III the coercive force Hc, respectively.

In general, material for a magnetic shield case, especially for a magnetic shield case of a magnetic head used for recording only, is required to have initial permeability  $\mu_0$ , greater than 3,000 and magnetic flux density B greater than 3,000 Gausse. Further, the coercive force Hc, must be selected smaller than 0.1 Oersted. Accordingly, in order to make the coercive force Hc smaller than 0.1, the amount x of Cr added to the alloy must be selected greater than about 6 weight percent, as is apparent from FIG. 6, which shows compositions of the ternary alloy containing no Mo. The fact that the addition of an amount x of Cr must be selected more than 6 weight percent may also be understood from, for example, FIG. 8 which shows the composition of a quaternary alloy  $(FeNi)CrMo$  and the rust forming characteristic thereof. That is to say, FIG. 8 illustrates the anti-corrosive characteristics of the quaternary alloy  $(FeNi)CrMo$ , in which the amounts of Cr and Mo contained therein are varied, respectively. In FIG. 8, values described in the vicinity of the circles represent an incremental ratio of weight per unit time when a sample is oxidized at temperatures of  $600^\circ C.$ , while the values in parentheses designate the decremental weight of a sample which is immersed in salt water of 8 percent for 100 hours. From FIG. 8 it will be observed that if the additional amount of Cr is smaller than 6 weight percent with respect to the total weight of the quaternary alloy, the rust forming rate K becomes greater than

ability  $\mu_0$ , magnetic flux density B and coercive force Hc thereof when the amounts of Cr and Mo in the quaternary alloy  $(FeNi)CrMo$  are changed. The upper, middle and lower numerals at marked points on this diagram represent the values of coercive force, magnetic flux density, and initial permeability, respectively, of alloys having compositions corresponding to such points. Since the initial permeability  $\mu_0$ , of material used for a shield case must be greater than 3,000 as mentioned above, it will be seen from FIG. 6 that the amount of Cr must be selected lower than about 12 weight percent with respect to the total amount of the quaternary alloy, while the amount of Mo must be selected higher than about 0.5 weight percent with respect to the total amount of the quaternary alloy. In this discussion, the amounts of Fe and Ni are assumed substantially equal in weight ratio. It is, however, observed similarly from FIG. 10, in which the weight ratio of Fe to Ni is made different, that if the amount of Mo is selected lower than 0.5 weight percent relative to the total amount of the quaternary alloy, its initial permeability  $\mu_0$ , is decreased.

FIG. 10 is a graph showing the magnetic characteristic of a quaternary alloy designated by  $(Fe_{60}Ni_{40})_{92-x}Cr_xMo_x$ , that is to say, the initial permeability  $\mu_0$ , magnetic flux density B and coercive force Hc thereof, when the amount x of Mo is changed in weight percent. From FIG. 10 it will be observed that when the amount of Mo is selected smaller than 0.5 weight percent, relative to the total amount of the quaternary alloy, its initial permeability  $\mu_0$ , is greatly increased. Similarly, when the amount of Mo is selected higher than 8 weight percent, its magnetic flux density B becomes lower than 3,000 (which is not shown but was ascertained by experiment). Further, the quaternary alloy thus obtained becomes uneconomical. Accordingly, in preferred embodiments of the magnetic alloy of the invention, the amount of Mo is selected lower than about 8 weight percent and greater than 0.5 weight percent.

Based upon the above results, the magnetic material or alloy of the present invention which mainly consists of  $(FeNi)CrMo$  is formulated to have a ratio of Ni to Fe (Ni/Fe) ranging from about 0.54 to about 1.5 weight percent, about 6 to about 12 weight percent of Cr and about 0.5 to about 8 weight percent of Mo. Such alloys are formed by conventional alloy techniques which include heat-treatment in a magnetic field and need no further explanation.

The following Table shows, by way of example, various characteristics of the conventional 79-Permalloy, 45-Permalloy and the magnetic material according to the present invention.

TABLE

|                        | 45-Permalloy | 79-Permalloy | $(Fe_{50}Ni_{30})_{90}Cr_xMo_2$ | $(Fe_{60}Ni_{40})_{90}Cr_xMo_2$ |
|------------------------|--------------|--------------|---------------------------------|---------------------------------|
| B[Gau $\beta$ ]        | 15000        | 7000         | 9070                            | 5500                            |
| $\mu_0$                | 3000         | 10000        | 15800                           | 18000                           |
| Hc[Oe]                 | 0.1          | 0.01         | 0.049                           | 0.03                            |
| K[mg $^2$ /Cm $^4$ hr] | 0.07         | 0.006        | 0.005                           | 0.01                            |

0.01 and tends to lower the anticorrosive characteristic of the alloy. In this discussion, it is assumed that Fe and Ni are substantially equal in weight.

FIG. 9 is a diagram showing the composition of a quaternary alloy  $(FeNi)CrMo$  and the initial permea-

From the above Table, it will be observed that the magnetic material of the present invention has magnetic characteristics B,  $\mu_0$ , Hc, equal to or higher than that of the 45-Permalloy and a rust forming rate K, substantially equal to that of the 79-Permalloy. Further, it

will be also understood that the magnetic material according to the present invention can be economically manufactured and economically worked or processed.

FIG. 11 shows a magnetic head 1 which is used for the wear test of the magnetic alloys according to the present invention. The magnetic head 1 consists of a shield case 2 provided with two windows 3 and two magnetic head cores 4 housed in the shield case 2. In this case, the magnetic head cores 4 are molded in the shield case 2 with a resin and both of the magnetic head cores 4 and the shield case 2 have the same tape contact surface.

FIGS. 12A to 12D, inclusive, are graphs showing worn states of the tape contact surface of magnetic heads after tape running tests, in which the materials for the shield case 2 and the magnetic head cores 4 of the magnetic head 1 shown in FIG. 11 were varied. In this test an ordinary magnetic tape was caused to travel in contact with the contact surface of the respective magnetic heads for 200 hours at a predetermined pressure. In the Figures, the dotted line shows the level of the contact surface of the magnetic head before the test.

FIG. 12A corresponds to the situation where both of the shield case 2 and the magnetic head cores 4 were both composed of 79-Permalloy. From FIG. 12A it will be apparent that the shield case 2 and the magnetic head cores 4 were substantially uniformly worn to a relatively large degree.

FIG. 12B corresponds to the situation where the shield case 2 was made of 79-Permalloy while the magnetic head cores 4 were made of hard Permalloy. In this situation, the magnetic head cores 4 were worn less but the shield case 2 was worn by similar amounts as that shown in FIG. 12A.

FIGS. 12C and 12D correspond to the situation where the shield case 2 was made of the magnetic alloys according to the present invention, in this example, the quaternary alloy (FeNi)Cr<sub>8</sub>Mo<sub>1</sub>, while the magnetic head cores 4 were made of the 79-Permalloy and hard Permalloy respectively. It will be apparent from FIGS. 12C and 12D that the shield case 2 made of the magnetic alloys according to the present invention is not only less worn but acts to protect the magnetic

5 head cores from being worn. In other words, the magnetic alloys of the present invention are most preferable when used in combination with a magnetic head. It may be possible to add one or more of the materials selected from the group consisting of niobium (Nb), titanium (Ti) and vanadium (V) to the quaternary alloys (FeNi)CrMo in a relatively small amount, for example, about 1 weight percent relative to the total amount of the alloy to enhance its hardness. In this situation, however, it should be noted that if the amount of such further additive exceeds 1 weight percent the permeability of thus obtained alloys becomes low and working thereof becomes rather difficult.

10 In the above discussion, the magnetic alloys according to the present invention were used as a magnetic shield case for a magnetic head, however, the alloys of the invention are also useful as a magnetic shield plate disposed between magnetic head cores.

15 It may also be possible that the magnetic alloys of the present invention can be used for ordinary magnetic shields.

20 It will be apparent that many modifications and variations may be effected without departing from the scope of the novel concepts of the present invention.

25 I claim as my invention:

1. A magnetically heat-treated alloy consisting essentially of iron, nickel, about 6 to about 12 weight percent chromium, and about 0.5 to about 8 weight percent molybdenum wherein a weight ratio of nickel to iron is in the range of about 0.54 to about 1.5, said alloy being characterized as having an initial permeability greater than 3,000, a magnetic flux density greater than 3,000 Gausses, a coercive force less than 0.1 and a rust-forming rate less than about 0.01.

30 2. A magnetically heat-treated alloy according to claim 1 and including less than about 1 weight percent of a material selected from the group consisting of niobium, titanium, vanadium and mixtures thereof.

35 3. A magnetically heat-treated alloy according to claim 1 wherein said alloy consists of (Fe<sub>50</sub>Ni<sub>50</sub>)<sub>90</sub>Cr<sub>8</sub>Mo<sub>2</sub>.

40 4. A magnetically heat-treated alloy according to claim 1 wherein said alloy consists of (Fe<sub>60</sub>Ni<sub>40</sub>)<sub>90</sub>Cr<sub>8</sub>Mo<sub>2</sub>.

45 \* \* \* \* \*